

Sept. 12, 1939.

W. HOSKINS, JR

2,172,873

HECTOGRAPH ROLL OR BLANKET

Filed Jan. 24, 1938



Inventor:  
William Hoskins Jr.  
By: Zabel, Carlson, Fitzbaugh & Wells  
Attorneys

## UNITED STATES PATENT OFFICE

2,172,873

## HECTOGRAPH ROLL OR BLANKET

William Hoskins, Jr., La Grange, Ill., assignor to  
Ditto, Incorporated, Chicago, Ill., a corporation  
of West Virginia

Application January 24, 1938, Serial No. 186,486

9 Claims. (Cl. 41—31.6)

The invention relates to hectograph rolls or blankets which usually comprise a backing and a layer of gelatinous material, the gelatinous material being secured to the backing by a suitable bonding agent, which preferably is of high clarifying power, so that the inks employed in the hectograph process will disappear rapidly.

The backing of a hectograph roll is usually paper or cloth, but my invention is limited to this type of backing only to the extent indicated by the appended claims.

To facilitate the disclosure of the invention, reference is made to the accompanying drawing, which is a cross-section through a hectograph band embodying the invention.

In the drawing the reference character 10 designates the backing of the improved hectograph band, the backing being preferably coated with an ordinary lacquer, such as, for example, pyroxelin lacquer, if the backing consists of paper or cloth. The lacquer is shown at 11 on both sides of the backing sheet, although it is generally customary to coat on one side only by means of a roller.

Applied to one side of the backing 10 and adhering to the lacquer coating 11 thereon is a bonding agent 12, to which the gelatinous mass 14 is applied.

In accordance with this invention, the improved bonding medium 12 is composed largely of glue and adsorbent filler. The preferred composition consists largely of ammonium caseinate, in combination with a colloidal adsorbent material such as bentonite or silica gel, with, if desired, a suitable water soluble plasticizer such as invert sugar, glycerine, or sulphonated oil. Addition of a tanning agent, such as chrome alum, ferric chloride, potassium dichromate, formaldehyde, tannic acid and the like may also be used to increase the penetration of the bond into the hectograph mass.

The following example of a preferred embodiment of the bonding agent is given by way of illustration:

| I                  | Parts by weight |
|--------------------|-----------------|
| Casein             | 10              |
| Ammonium hydroxide | 5               |
| Bentonite          | 5               |
| Invert sugar       | 30              |
| Water              | 125             |

In using this composition on a pyroxaline coated cloth I find it advantageous to add say ten to twenty per cent of a cellulose solvent such as diethylene glycol or the mono-ethyl-ether of

ethylene glycol to provide a better adhesion to the cloth itself.

Additional examples of bonding agent formula:

| II           | Parts by weight |
|--------------|-----------------|
| Glue         | 10              |
| Water        | 115             |
| Bentonite    | 5               |
| Invert sugar | 30              |
| Glycerine    | 30 10           |

| III       | Parts by weight |
|-----------|-----------------|
| Glue      | 10              |
| Water     | 115 15          |
| Bentonite | 5               |
| Glycerine | 30              |

Numerous changes can be made in the above process without departing from the scope of my invention and it is understood that the detailed example given above is to be interpreted as illustrating and not limiting the scope of my invention. Other colloidal adsorbent materials than bentonite and silica gel can be used. However, I prefer to use the colloidal clays of which bentonite is a good example. These materials, particularly when used with casein glues, give an especially satisfactory adhesion. Moreover, the materials appear to act as clarifying agents, aiding in the removal of excess dye from the hectograph composition.

What I claim as new is:

1. A duplicating sheet comprising a flexible backing, a layer of hectograph composition applied to said backing, and means for securing said hectograph composition to said backing comprising an adhesive containing an adsorbent inorganic colloidal material.

2. A duplicating sheet comprising a flexible backing, a layer of hectograph composition applied to said backing, and means for securing said hectograph composition to said backing comprising a colloidal clay.

3. A duplicating sheet comprising a flexible backing, a layer of hectograph composition applied to said backing, and means for securing said hectograph composition to said backing comprising bentonite.

4. A duplicating sheet comprising a flexible backing, a layer of hectograph composition applied to said backing, and means for securing said hectograph composition to said backing comprising an adhesive containing casein and an adsorbent inorganic material.

5. A duplicating sheet comprising a flexible backing, a layer of hectograph composition applied to said backing, and means for securing said hectograph composition to said backing comprising an adhesive containing casein and a colloidal clay.
6. A duplicating sheet comprising a flexible backing, a layer of hectograph composition applied to said backing, and means for securing said hectograph composition to said backing comprising an adhesive containing casein and bentonite.
10. 7. A method of making duplicating sheets comprising the steps of coating a backing with a

bonding agent containing inorganic adsorbent colloidal material and applying a layer of the hectograph composition to the bonding agent.

8. A duplicating sheet comprising a flexible backing having an adhesive coating thereon comprising bentonite and a protein adhesive, and a hectograph composition secured to said backing by said adhesive coating.

9. A duplicating sheet comprising a flexible backing, a layer of hectograph composition applied to said backing, and means for securing said hectograph composition to said backing comprising silica gel.

WILLIAM HOSKINS, JR.